

Jan. 27, 1953

E. MARBURG

2,626,436

INGOT MOLD

Filed Sept. 18, 1951

2 SHEETS—SHEET 1



**FIG. 10.**

K-87  
Inventor:  
EDGAR MARBURG,  
by: Donald G. Dalton  
his Attorney.

Jan. 27, 1953

E. MARBURG  
INGOT MOLD

2,626,436

Filed Sept. 18, 1951

2 SHEETS—SHEET 2



*Inventor:  
EDGAR MARBURG,  
by Donald G. Dalton  
his Attorney.*

## UNITED STATES PATENT OFFICE

2,626,436

## INGOT MOLD

Edgar Marburg, Pittsburgh, Pa., assignor to  
United States Steel Company, a corporation of  
New Jersey

Application September 18, 1951, Serial No. 247,047

5 Claims. (Cl. 22—139)

1

This invention relates to improvements in ingot molds.

Molten steel in an ingot mold solidifies inwardly from the mold wall at an extremely rapid rate initially. The rate of solidification decreases sharply to a depth of about  $1\frac{1}{2}$  inches; beyond this latter depth it is relatively low and decreases slowly. Mathematically solidification follows Feild's equation,  $d=k\sqrt{t}$ , in which  $d$  is the solidified depth in inches,  $t$  is the time in minutes, and  $k$  is a constant. The value of  $k$  varies from about 0.75 to 1.00, increasing with increase in mold wall thickness and with decrease in ingot width. The  $k$ -value increases in this fashion because in ingot molds, where the wall thickness is at least 2 inches, a much larger proportion of the extracted heat is absorbed in heating the mold walls than is lost by radiation. The thicker the wall, the more heat extracted and the more rapid the rate of solidification. For the same reason solidification is more rapid from the corners of an ingot of rectangular cross section than from the sides, the corners being subject to heat extraction by two adjacent mold walls.

In solidifying, steel contracts about 4 per cent in volume, in cooling from the solidus temperature to room temperature, the solid metal contracts an additional 7 per cent. Thus, as solidification proceeds inwardly, the solid wall continuously contracts in volume as it loses temperature. Following solidification of the outer shell, subsequent contraction of the metal toward the interior of the ingot must be greater than that of the outer shell. Hence the internal volume of the solidifying ingot shell is constantly enlarging with respect to the volume of the contained liquid metal. As a result the surface of the liquid metal drops continuously during solidification, and a void or pipe, whose shape approximates an inverted cone, is formed in the middle of the ingot. Pipe may extend downwardly to mid-height or even lower in an ingot. Metal may solidify completely across an ingot at one or several levels near the top; such solidification is referred to as bridging. Pipe cavity above bridging, or pipe that is free from bridging is referred to as primary or open pipe; pipe cavity below bridging is designated secondary pipe. As the latter type of pipe is protected against oxidation, its surfaces may be welded together when the ingot is rolled. Because primary pipe is subject to oxidation by contact with the air, however, its surfaces cannot be welded effectively by rolling; hence primary pipe may result in so-called lamination in the rolled product. Depending upon the application, a greater or less

2

extent of the upper portion of the rolled bloom containing primary pipe is cropped, that is, it is sheared off and rejected as scrap metal.

To minimize pipe in killed-steel ingots, hot tops or collars of refractory insulating material (generally fireclay), which extend variably 2 to 3 inches inside the mold (depending upon the weight of ingot desired), are placed on molds prior to casting ingots therein. In the casting of ingots, liquid metal is teemed from a ladle to fill the mold and the superimposed hot top; the metal contained in the latter is referred to as the sinkhead. The hot top conserves heat so that the sinkhead metal does not freeze so rapidly as does the metal next to the mold wall. By maintaining a reservoir of liquid metal sufficient to compensate for all of the contraction in the ingot body, the hot top causes all of the pipe cavity to be confined to the sinkhead. After the ingot is rolled to a bloom or slab, the sinkhead portion is cropped, and rejected as scrap. With use of a hot top, sound steel can be obtained below about 15 per cent top discard; without a hot top, the top discard necessary to eliminate pipe may be 35 per cent or more of the total ingot weight.

It has long been recognized as desirable that heat be extracted more rapidly from the bottom portion of a solidifying ingot than from the top portion. Desirably the bottom portion solidifies completely while there is still a relatively wide column of liquid metal in the top portion. Final solidification of the liquid column in the middle of an ingot proceeds rapidly in a vertical direction. The face of vertical solidification approximates a modified V-shape, with a rounded lower portion in any vertical section. The angle of the V as it approaches the top of an ingot is a criterion of the internal soundness of the ingot. If this V-angle is sufficiently wide, segregated material diffuses effectively into the sinkhead and the interior of the ingot is sound; that is, it is substantially free from pipe and porosity. If on the other hand the V-angle is sharp, segregation and porosity are much more liable to develop in the upper middle portion of the ingot. If the V does not reach the top, that is, if bridging occurs, secondary pipe and axial porosity invariably develop below the bridging.

To secure favorable solidification from the base upwardly, mold walls taper upwardly and commonly are 2 or 3 inches thicker at the base than at the top. For example, the wall of a 24 by 24 inch mold may be 5 inches thick at the top and  $7\frac{1}{2}$  inches thick near the base. Numerous experiments in which ingots cast in molds with

tapered walls have been dumped at various times after pour, and the thickness of the solidified shells measured, however, reveal that mold taper is ineffective for the purpose intended. From these experiments it has been determined that the face of solidification is always substantially parallel to the mold wall; that is, solidification does not proceed more rapidly from the thick base than it does from the thin top of a tapered mold wall. The reason appears to be that the thin upper portions of the mold heat to higher temperatures than do the thick lower portions. Thus temperature gradients are established, which cause heat to flow downwardly in the mold walls. As a result of this heat flow, the normally slower solidification rates adjacent to the thin upper walls are accelerated, whereas the normally faster solidification rates adjacent to the thick lower walls are retarded. Thus downward heat flow from the thin to the thick end of a uniformly tapered mold wall equalizes solidification rates throughout the height of the mold.

An object of the present invention is to provide improved ingot molds which effectively produce a desirable solidification pattern in the ingot, that is, the ingot solidifies transversely more rapidly across the bottom portion than it does across the top portion, and the solidifying surface advances vertically as a wide-angled V, centered on the vertical axis.

A further object of the invention is to provide improved ingot molds of a wall configuration which accelerates transverse heat extraction from the bottom portion of a solidifying ingot and decelerates transverse heat extraction from the top portion, which procedure is favorable to the production of sound ingots.

In accomplishing these and other objects of the invention, I have provided improved details of structure, preferred forms of which are shown in the accompanying drawings, in which:

Figure 1 is a top plan view of an ingot mold which embodies features of the present invention;

Figures 2 and 3 are vertical sectional views of the mold taken on lines II-II and III-III respectively of Figure 1;

Figure 4 is a horizontal sectional view of the mold taken on line IV-IV of Figure 2;

Figure 5 is a top plan view of a modified ingot mold which also embodies features of the invention;

Figures 6 and 7 are vertical sectional views of the modified mold taken on lines VI-VI and VII-VII respectively of Figure 5;

Figure 8 is a horizontal sectional view of the modified mold taken on line VIII-VIII of Figure 6; and

Figures 9, 10 and 11 are schematic plan and horizontal sectional views to illustrate the manner in which the constant  $k$  changes with different proportioning of the sides and corners in a 24 by 24 inch mold having side walls 5 inches thick.

In the embodiment of the invention shown in Figures 1 to 4 the mold is of substantially square cross section and has a bottom 10, side walls 12 and corner walls 13. The side walls are of substantially uniform thickness throughout their height, although if desired, they can have the usual vertical corrugations. The corners taper upwardly in longitudinal section, so that at the base, they are much thicker than the sides, at the top somewhat thinner, and at an intermediate height of the same thickness.

When molten metal is introduced into this mold, the side walls 12 are quickly heated. Near the base a temperature gradient develops between the hot side walls and the enlarged corner walls 13, which latter are relatively cool. As a result of this gradient, the  $k$ -value for transverse solidification is much greater than it would be in a mold of uniform wall thickness. As the corner thickness decreases upwardly, the  $k$ -value for solidification also decreases. At the height where the sides and corners are of the same thickness, the rate is similar to that in a conventional ingot mold, where the sides and corners are of equal thickness in any transverse section. Above this height the ratio of corner to side thickness decreases progressively below unity. Hence the efficacy of corners as chills decreases to practical disappearance at the top of the mold. Thus the  $k$ -value for solidification across the top of the ingot is less than that for an ingot cast in a mold of uniform wall thickness, and is considerably less than the  $k$ -value for solidification across the base of the same ingot.

Heat flow throughout a mold constructed as shown in Figures 1 to 4 may be considered in comparison with that in a mold of conventional design. As discussed previously, undesirable downward heat flow occurs in conventional molds with tapered walls. As the side walls of the mold shown in Figure 2 are of uniform thickness, no temperature gradients are established therein; hence there is no tendency for heat to flow downwardly. In a conventional mold, such as Figure 10 shows schematically, the corners are of the same thickness as the sides, or at least bear a constant ratio thereto; hence the effect of the corners on heat extraction at the middle plane does not vary greatly throughout the height of the mold. Because of the continually varying ratio of corner thickness to side thickness in the mold shown in Figure 3, however, the tendency for heat to flow from the middle of a side to a corner is maximum near the base, minimum at the top, and varies uniformly between these sections. Thus this mold is advantageously designed to cause increased rates of heat extraction, hence faster solidification near the base than across the top of an ingot.

As the wall thickness at the corners of the mold, shown in Figure 3 increases downwardly, there is a tendency for heat to flow downwardly in the mold corners, which downward heat flow is detrimental to the effectiveness of the mold. As the temperatures at mold corners are considerably lower than those at the middles of the sides of molds, however, the longitudinal gradients in the corners are considerably smaller than the transverse gradients from the middles of the sides to the corners. Further the longitudinal gradients are much longer than the transverse gradients. Hence the unfavorable downward heat flow in the corners is considerably smaller than the transverse heat flow from the middles of the sides to the corners, so that the effectiveness of this mold is diminished only slightly by downward heat flow at the corners.

Figures 5 to 8 show a modification. The cross sections at the top, near the middle, and at the base are similar to the corresponding sections of the mold shown in Figures 1 to 4. The distinctive feature of the modified mold is in the shape of the outer surface of the corners. This surface does not taper continuously as in Figure 3, but the taper in the upper and lower portions, designated 18 and 19 respectively, is considerably

less or none at all, and that in an intermediate portion 20, considerably greater. Heat extraction from an ingot cast in a mold constructed as shown in Figures 5 to 8 is generally similar to that described for Figures 1 to 4. However, the volume of mold metal in the upper portion of the mold shown in Figures 5 to 8 is less and that in the lower portion greater than the volumes of corresponding portions of the mold in Figures 1 to 4; consequently the difference in heat extraction rates between the top and the bottom is greater in the mold in Figures 5 to 8.

The present invention has been illustrated as applied to a big-end-up mold, but all the principles thus far described are applicable as well to big-end-down molds. However, in big-end-up molds the effect of the base 10 on heat extraction by the side walls requires consideration. The base of a big-end-up mold is normally thicker than the side walls; hence the temperature of the base during the solidification of an ingot is lower than that of the side walls. Thus heat flows from these walls downwardly into the base, just as heat flows transversely from the hotter middles of the sides to the colder corners. It has been mentioned that downward heat flow in tapered mold walls is disadvantageous. In walls of uniform thickness, such as the side walls 12, however, a temperature gradient develops first only at the extreme lower portion of the wall. As solidification continues, this gradient proceeds upwardly, but it is always stronger in lower portions of the mold. Thus the effect of a closed base in conjunction with side walls of uniform thickness is to cause solidification to proceed desirably from the base to the top of an ingot. The heavier the base, the more effectively it performs this function. For this reason, the bottom 10 in both mold constructions illustrated has been widened to the same widths as the corners, as indicated at 22. The widened portion can be of any height up to height of the center of the hemispherical portion at the bottom of the mold cavity. Big-end-down molds may be similarly thickened in the lower portion of their sides up to about a third of their height.

From the foregoing description it is seen that the present invention affords an improved ingot mold that assures that the bottom portion of an ingot solidifies transversely at a faster rate than does the top portion. The mold not only accelerates cooling of the bottom portion of the ingot, but actually decelerates cooling of the top portion.

While I have shown and described only certain preferred embodiments of the invention, it is apparent that other modifications may arise. Therefore I do not wish to be limited to the disclosure set forth but only by the scope of the appended claims.

I claim:

- An ingot mold of substantially rectangular cross section in which the side walls are of substantially uniform thickness from bottom to top and the corner walls are of greater thickness than the side walls adjacent the bottom to accelerate solidification of an ingot in this portion of the mold, and of less thickness than the side walls adjacent the top to decelerate solidification in this latter portion, as compared with solidification rates of an ingot cast in a mold of uniform wall thickness in transverse section equal to the thickness of the side walls of the described mold.
- An ingot mold of substantially rectangular cross section in which the side walls are of substantially uniform thickness from bottom to top and the corner walls taper upwardly and are of greater thickness than the side walls adjacent the bottom so that they can extract heat from the side walls to accelerate solidification of an ingot in this portion of the mold and are of less thickness than the side walls adjacent the top to retard solidification in this latter portion, as compared with solidification rates of an ingot cast in a mold of uniform wall thickness in transverse section equal to the thickness of the side walls of the described mold.
- An ingot mold as defined in claim 2 in which the corner walls in longitudinal section taper substantially uniformly throughout their height.
- An ingot mold as defined in claim 2 in which the corner walls in longitudinal section taper but slightly in their top and bottom portions and taper abruptly in their intermediate portions.
- A big-end-up ingot mold of substantially rectangular cross section in which the side walls are of substantially uniform thickness from bottom to top, the corner walls are of greater thickness than the side walls adjacent the bottom to accelerate solidification of an ingot in this portion of the mold and of less thickness than the side walls adjacent the top to decelerate solidification in this latter region, and the bottom of the mold extends outwardly below the side walls to further accelerate solidification in the bottom portion, as compared with solidification rates of an ingot cast in a mold of uniform wall thickness in transverse section equal to the thickness of the side walls of the described mold.

EDGAR MARBURG.

#### REFERENCES CITED

- 55 The following references are of record in the file of this patent:

#### UNITED STATES PATENTS

- |              |       |              |
|--------------|-------|--------------|
| Number       | Name  | Date         |
| 60 1,758,823 | Bloge | May 13, 1930 |